

J. M. LYNCH.  
METHOD OF HARDENING AND TEMPERING STEEL.  
APPLICATION FILED APR. 23, 1909.

1,029,877.

Patented June 18, 1912.



WITNESSES  
Edith C. Hollbrook  
Elizabeth C. Coupe

INVENTOR  
John M. Lynch  
By his Attorney,  
Nelson W. Howard

# UNITED STATES PATENT OFFICE.

JOHN M. LYNCH, OF BEVERLY, MASSACHUSETTS, ASSIGNOR TO UNITED SHOE MACHINERY COMPANY, OF PATERSON, NEW JERSEY, A CORPORATION OF NEW JERSEY.

## METHOD OF HARDENING AND TEMPERING STEEL.

1,029,877.

Specification of Letters Patent. Patented June 18, 1912.

Application filed April 23, 1908. Serial No. 491,732.

To all whom it may concern:

Be it known that I, JOHN M. LYNCH, a citizen of the United States, residing at Beverly, in the county of Essex and State 5 of Massachusetts, have invented certain Improvements in Methods of Hardening and Tempering Steel, of which the following description, in connection with the accompanying drawings, is a specification, 10 like reference characters on the drawings indicating like parts in the several figures.

This invention relates to methods of hardening and tempering steel and particularly to a method of partially hardening 15 steel tools or other articles of substantially uniform composition throughout.

In the following description and claims the term "tool" will frequently be used to designate the article to be hardened, but it 20 will be understood that by the use of this term it is not intended to restrict the invention to hardening and tempering steel articles properly designated as tools, and that the invention may be applied equally to 25 hardening and tempering any articles of like material to which it is desired to give the characteristics which this method is especially adapted to give.

An object of the invention is an improved 30 method of hardening and tempering steel tools, or other articles of substantially uniform composition throughout, by which a tool may be produced which is hardened the desired distance back from its operating 35 edge, without a sharp line of demarcation between the hardened and unhardened portions. By such a method the strains usually left along this line in partially hardened tools, which have been hardened and 40 tempered by ordinary methods, may be avoided and all-steel tools, having high shock resisting qualities and tempered to meet the requirements of the work which they are to perform, may be produced.

Another object of the invention is a 45 method of hardening and tempering by which a tool, having an operating edge of a particular contour, may be partially hardened in the manner above specified without 50 affecting the contour of said edge.

A further object of the invention is a method of hardening and tempering tools, especially applicable to tools of the kind just described, by which a tool may be har-

dened and tempered in the desired parts 55 without the necessity of raising the entire tool to the hardening temperature.

With the foregoing and other objects in view, the method of this invention has been devised.

The invention comprises in one of its important aspects a method of hardening and tempering tools which consists in simultaneously heating different parts of the tool in mediums so arranged and of such relative 60 conductivity that the part of the tool to be hardened is heated to the desired hardening temperature and that the adjacent part is heated decrementally from the part to be hardened back and then immersing said 65 tool while thus heated in a suitable hardening bath.

More specifically the invention comprises that improvement in the art of hardening and tempering tools of uniform composition 70 throughout which consists in immersing the part of the tool to be hardened in a metallic heating bath covered with a layer of heat conducting material of a depth and of a conductivity so related to the size and carbon content of the particular tool to be hardened that said tool will be heated decrementally from the immersed portion 75 back, and then immersing said tool in a hardening bath.

As above suggested, the method of this invention is especially applicable to the hardening and tempering of tools having operating edges of predetermined contours and in practice it has been found especially 80 useful in the hardening and tempering of stock cutting dies, such, for example, as those used with the upper cutting machine known to the trade as the clicking machine.

For convenience of description and illustration the invention will be herein represented as applied to the hardening and tempering of dies of the type above referred to. These dies are of irregular shape, being 85 designed to cut the different parts of the uppers of boots or shoes, and are provided with cutting edges which form closed outlines. Each die is usually provided also with a back lying in one plane to receive the cutting pressure. It is desirable that the 90 cutting edges of these dies be comparatively hard and that the back, which is to receive the cutting pressure, or in the usual prac-

tice, the cutting blow, be comparatively soft or tough. Difficulty has been experienced in the past in producing dies having these characteristics. One practice has been to 5 make the die of stock composed of two different materials so arranged that the hard material would form the cutting edge and the soft material would form the blow receiving part of the die. Even with stock 10 of these characteristics difficulty has been found in hardening and tempering the cutting edge of the die, after it has been shaped to the pattern to be cut, without distorting said edge and thereby causing it to depart 15 from the pattern.

The usual method of hardening and tempering these dies has involved heating the entire die to the hardening temperature. This practice is objectionable since internal 20 strains are apt to be left in the die from its shaping operations and when the die is thus subjected to a high heat and sudden cold, it is impossible to foretell what the effect of these strains will be upon the final shape of 25 the die. The reshaping of the die after the hardening and tempering operations has therefore involved considerable labor and skill. Die making up to the present time has been a comparatively skilled art, re- 30 quiring high priced labor, and one of the principal elements of skill involved has been, as above suggested, that required to reshape the die after it had been distorted by the hardening and tempering process.

35 An important feature of the present invention is the novel heating step by which only that portion of the die which is to be hardened is heated to the hardening temperature while the remaining portions of 40 the die are heated decrementally from the portion brought to the hardening temperature, the heating being so graduated that no sharp line of demarcation between the hardened and unhardened portions of the 45 die is left. By the methods heretofore employed in hardening dies it has been difficult to avoid the formation of the line just referred to. Where it has been attempted to partially harden a tool by heating only the 50 portion to be hardened to the hardening temperature, this line has still been formed, since the portion of the tool not to be hardened has been kept at a temperature considerably below that of the part to be hardened, whereby near the line between the two 55 parts there would be a sharp change in the internal structure of the tool, thus causing the tool frequently to break at this point in use, even if cracks were not formed during 60 the hardening operation. In other methods it has been attempted to effect a differential hardening of the tool by heating the entire tool to the hardening temperature and then quenching only the part of the tool which 65 is to be hardened, letting down the hardness

by the heat conducted from the unquenched portion and then completing the cooling. This practice is as objectionable as that above referred to since the same sharp line is left between the hardened and unhardened portions of the tool as when the first described method is employed, and, furthermore, when the edge to be hardened has been given a desired outline this outline will usually be distorted, as above pointed out. 70

75 By the method of this invention the formation of the sharp line of demarcation between the hardened and unhardened portions of the tool is avoided by simultaneously heating different parts of the tool in 80 mediums so arranged and of such relative conductivity that the part of the tool to be hardened is heated to the desired hardening temperature, which is preferably the highest transforming point of the steel employed, and that the adjacent part receives a heat which gradually diminishes from the first mentioned part or, in other words, the tool is heated decrementally from the part 85 to be hardened.

90 The method will now be described with especial reference to its application to hardened and tempering shallow open dies of the type employed with the clicking machine.

95 In the accompanying drawings,—Figure 1 illustrates suitable heating means for carrying out the method of this invention; Fig. 2 illustrates a convenient arrangement of the quenching or hardening bath for use 100 in carrying out the method of this invention.

The dies are preferably made of steel of uniform composition throughout and the method will be specifically described with 105 reference to its application to the hardening and tempering of dies made from selected billets of uniform open-hearth steel in which the accidental or injurious admixtures of phosphorus, sulfur, copper, arsenic, 110 etc., are kept well below .05 per cent. in each case and in which the carbon content, from .60 per cent. to .90 per cent, preferably .80 per cent., is sufficient to give the required edge holding capacity and, also, when tempered in oil, after having been hardened by the method of this invention, the highest possible shock resisting qualities. The manganese content of the steel, from .30 per cent. to .50 per cent. is proportioned to 115 give the highest possible welding power and also to exert the greatest influence on the change in volume and shape of the steel when hardened, thus preventing shortening 120 of the outline of the dies.

125 The dies having been made from steel of the composition above indicated, preferably by the method disclosed in United States Letters Patent No. 922,926 granted May 25, 1909, to J. M. Lynch for improvements in 130

methods of making dies are brought to the tempering room and are then heated in the following manner. The die being dry is floated edge down upon a heating bath composed of molten lead covered with a layer of charcoal of such a depth that the heat of the bath may be conducted to the part of the die adjacent to the part to be hardened to such an extent that said part will be heated decrementally from the part to be hardened back. A convenient bath is illustrated in Fig. 1.

In a suitable metallic receptacle 2, supported upon the brick lined frame 4 is a lead bath 6 covered with a layer of charcoal 8. A suitable grade of charcoal for covering the bath is what is known as P size charcoal, obtained from wood alcohol works. The bath is raised to the desired temperature by any suitable heating means, that herein illustrated comprising a burner 10 for an oil flame to which oil is fed through a pipe 12 controlled by a valve 14, compressed air being conducted to the burner through another pipe 16 and controlled in amount by a valve 18. The lead bath is heated to a temperature somewhat higher than the highest transforming point of the steel in order that the part of the die to be hardened may be quickly raised to the desired temperature, and in tempering dies made of steel of the composition above indicated, the bath is preferably raised to a temperature of 1550° F. which is preferably controlled by a pyrometer, the highest transforming point of the steel being approximately 1500°. When hardening dies of the type employed with the clicking machine, which are comparatively light and about  $\frac{1}{4}$  of an inch in height, the charcoal layer 8 is preferably of such a depth that only the upper edge or back of the die is exposed when the die is floated upon the bath. This edge is left exposed to permit the operator to locate the die when he wishes to remove it from the bath. These dies when thus floated upon the bath will be immersed about  $\frac{3}{16}$  of an inch.

The charcoal layer 8 has numerous functions, among which are to keep the surface of the lead from oxidizing and to form a blanket by which the temperature of the bath, near its upper surface, may be kept high, the heat conductivity of the charcoal, as is well known, being less than that of the lead. The principal function of the charcoal covering, however, in the present method, is to prevent wide variations in the temperature between adjacent portions of the die and particularly to prevent a marked variation in the temperature between the immersed portion and the portion lying outside the lead bath. This function the charcoal covering performs very satisfactorily when it is made of a suitable depth since by conduction it causes the temperatures to which different

parts of the dies are heated to vary gradually from the part to be hardened toward the back or striking surface, whereby no sharp change in the internal structure occurs in any part of the die from the part to be hardened back to the striking surface which is left in an unhardened condition. There is thus no sharp line of demarcation between the hardened and unhardened parts of the die as in dies hardened and tempered by ordinary methods.

The die shown at 20 in Fig. 1, having been floated upon the lead bath long enough to bring the part to be hardened, which includes its cutting edge, to the desired temperature, this being, as above suggested, preferably 1500°, is then taken from said bath and immersed in the quenching or hardening bath, preferably oil, which may be contained in any suitable receptacle, such for example, as that shown at 22 in Fig. 2. In practice this receptacle comprises the tank 22 containing cotton seed oil 24 which is kept stirred up and at a uniform temperature by jets of air taken preferably from a source of compressed air conducted down to the bottom through a pipe 26.

After the die has been heated and hardened in the manner described, the hardness is "let down" or tempered in the following manner. The die is taken from the hardening bath and immersed in an oil bath with a thermometer attachment, said bath being at a comparatively low temperature at the time the dies are placed in it, for example, at a temperature of about 200°. The die, or dies, is then heated to the desired reducing temperature which in the case of dies made of steel of the composition above indicated and for the purposes for which these dies are intended is preferably 540°. After the temper has thus been "let down" the dies are removed from the tempering bath and immersed in a cleaning bath consisting of a solution of caustic potash maintained at a temperature just below the boiling point by a thermostatic attachment. Immersion of the dies in this bath prevents too sudden cooling after they are removed from the tempering bath. After the dies have been washed in the caustic potash bath, they are taken out and permitted to cool to the temperature of the room. The oil used in the tempering bath is preferably beef tallow.

With dies of the sizes and composition above indicated the heating operation in the lead bath takes usually from 15 to 20 seconds. It will therefore be seen that this method may be carried out very quickly and very easily and with an assurance of substantially uniform results. The floating of the die upon the lead bath insures heating it back from its cutting edge to the hardening temperature a substantially uniform dis-

tance throughout the extent of said edge. It will therefore be seen that this method is especially useful in hardening and tempering tools having cutting edges which form closed outlines especially where the cross section of the tool is uniform throughout its outline. The method may also be used to advantage in hardening other kinds of tools and, in fact, is thus employed. The depth 5 of the layer of charcoal required to insure decremental heating from the part to be hardened back will vary of course with the size and carbon content of the tool to be hardened, the required hardening temperature 10 varying with the carbon content of the steel. When the distance from the operating edge of the tool to the back is comparatively great, it will not be necessary to carry the charcoal layer up to the back of the 15 tool.

It will be noted that an important advantage of this method when it is employed for hardening and tempering dies of the type above described is that in heating the die it 20 may be floated upon the heating bath and that thereby the dimensions of the part of the die which is to be raised to the hardening temperature will be automatically determined. It will therefore be noted that the 25 method contemplates heating a tool, having a cutting edge which forms a closed outline by floating the tool upon a heating bath having a specific gravity so related to the specific gravity and structure of the tool that 30 the part of the tool to be raised to the hardening temperature will be automatically immersed in the bath by the weight of the tool floating thereon.

Having described my invention, what I 40 claim as new and desire to secure by Letters Patent of the United States is:—

1. That improvement in the art of hardening and tempering tools which consists in simultaneously heating different parts of the 45 tool in different contiguous heat conducting mediums so arranged and of such relative conductivity that the part of the tool to be hardened is heated to the desired hardening temperature and that the adjacent part is heated decrementally from the part to be hardened, and then entirely removing said tool from the heat conducting mediums and immersing it forthwith in a hardening bath.
2. That improvement in the art of hardening and tempering tools of substantially 55 uniform composition throughout which consists in simultaneously heating different parts of the tool in different contiguous heat conducting mediums so arranged and of such relative conductivity that the part of the tool to be hardened is heated to the highest transforming point of the steel of which the tool is composed and that the adjacent part is heated decrementally from said first 60 mentioned part, and then entirely removing

said tool from the heat conducting mediums and immersing it forthwith in a hardening bath.

3. That improvement in the art of hardening and tempering tools of uniform composition throughout which consists in immersing the part of the tool to be hardened in a metallic heating bath covered with a layer of heat conducting material of a depth and of a conductivity so related to the size and carbon content of the particular tool to be hardened that said tool will be heated decrementally from the immersed portion and then immersing said tool in a hardening bath. 70

4. That improvement in the art of hardening and tempering tools of substantially uniform composition throughout, which consists in immersing the part of the tool to be hardened in a lead heating bath covered with a layer of charcoal of a depth sufficient to conduct the heat of the bath to the tool decrementally from the part immersed and then immersing the entire tool in a hardening bath. 75

5. That improvement in the art of hardening and tempering tools which consists in immersing the part of the tool to be hardened in a lead heating bath covered with a layer of charcoal extending to the upper 90 edge of the part of the tool not immersed whereby said tool is heated decrementally from the immersed portion, and then quenching said tool by immersing it in a hardening bath. 95

6. That improvement in the art of hardening and tempering tools of uniform composition throughout, which consists in heating the part of the tool to be hardened to the highest transforming point of the steel of 105 which the tool is composed by immersing said part in a metallic heating bath which is covered with a layer of heat conducting material of a depth and of a conductivity so related to the size and carbon content of the particular tool to be hardened that said tool will be heated decrementally from the immersed portion, immersing said tool in a hardening bath and then heating said tool in oil to temper it. 110

7. That improvement in the art of tempering tools, especially applicable to tempering tools having cutting edges which form closed outlines, which consists in floating the tool edge down upon a metallic heating bath covered with a layer of material of lower heat conductivity than the bath and of less specific gravity than the tool, the depth and heat conductivity of said layer of material being sufficient to insure that the 120 tool is heated decrementally from its immersed portion, and then immersing said tool in a tempering bath. 125

8. That improvement in the art of tempering dies, especially applicable to temper- 130

ing dies having cutting edges which form closed outlines, which consists in floating the die edge down upon a bath of molten lead covered with a layer of charcoal extending 5 to the upper edge of the die, whereby the die is heated for a short distance back from its cutting edge to the desired hardening temperature, the heat gradually decreasing to the upper or striking surface of the die, 10 with no sharp line of demarcation between the part raised to the hardening temperature and the remaining portions, and then immersing said die in a hardening bath.

9. That improvement in the art of hardening and tempering tools having cutting edges which form closed outlines and having substantially uniform cross-section, which consists in floating the tool edge down upon a heating bath of a specific gravity so 20 related to the specific gravity and structure of the tool that the part of the tool to be hardened will be automatically immersed in the bath by the weight of the tool floating thereon while the remaining portion will be 25 kept at a temperature sufficiently below that of the immersed portion to maintain the outline of the edge, and then immersing said tool in a hardening bath.

10. That improvement in the art of hardening and tempering tools, especially applicable to hardening and tempering tools having cutting edges which form closed outlines, which consists in floating the tool edge down upon a metallic heating bath covered with a layer of material of lower heat conductivity than the bath and of less specific gravity than the tool, the specific gravity of the bath being so proportioned to the specific gravity and structure of the tool that the part of the tool to be hardened will be 30 automatically immersed in the bath by the weight of the tool floating thereon and the depth and heat conductivity of the covering material being such that the tool will be heated decrementally from the immersed portion, whereby the tool may be allowed to remain stationary during the heating operation, and then immersing said tool in a 35 hardening bath.

In testimony whereof I have signed my 40 name to this specification in the presence of two subscribing witnesses.

JOHN M. LYNCH.

Witnesses:

H. DORSEY SPENCER,  
LEONARD M. JOHNSON.